

March 19, 1935.

H. SCHAGRIN

1,995,192

CLEANING IRON OR STEEL

Filed June 4, 1931



INVENTOR.  
HARRY SCHAGRIN.

BY

  
ATTORNEY.

## UNITED STATES PATENT OFFICE

1,995,192

## CLEANING IRON OR STEEL

Harry Schagrin, Oak Park, Ill., assignor, by  
mesne assignments, to Robert L. Kahn

Application June 4, 1931, Serial No. 542,007

5 Claims. (Cl. 204—1)

This invention relates to a process for cleaning iron or steel, and particularly for the removal of scale formed during annealing or hardening. In the manufacture of hardened steel parts, it is customary to have the steel in a soft condition during processing, and thereafter harden the steel in a suitable furnace and grind or polish the steel to final form. Also, it is customary to anneal cast iron to form soft iron. In the commercial manufacture of such parts, a hard scale is usually formed in the furnace, and if not removed prior to grinding or polishing, would result in the serious wear of such grinding equipment.

While numerous processes purport to remove scale, it has been found that such processes either appreciably etch the iron or steel during the removal of the scale or fail to completely remove the scale, particularly in inaccessible places caused by the drilling of recesses, and the like.

An object of this invention is to devise a simple, economical and speedy process for the removal of scale in such manner as to avoid the above objections.

The drawing is a diagrammatic showing illustrative of the steps in the process.

As actually applied, iron or steel covered with scale is made the cathode in a sulphuric acid solution. This solution has preferably between 10 and 15 per cent acid, and contains as an anode a material like lead, which is substantially insoluble in the electrolyte. The temperature of the bath is maintained between 110 and 120 degrees Fahrenheit—preferably 120 degrees Fahrenheit—while the current density is maintained at between 50 and 60 amperes per square foot of cathode. It has been found that the average scale is completely removed in from 6 to 12 minutes.

The iron or steel is removed from the bath, and in this condition has a dark-colored appearance. It is washed in water to remove the acid, and is then made the anode in a bath for brightening the surface. This bath is preferably alkaline and comprises about 2 to 8 ounces of sodium hydroxide or other alkali, and between 2 and 4 ounces of trisodium phosphate per gallon of water. The trisodium phosphate may be omitted, if desired, but better results are secured with it. The cathode is preferably of iron, although any other insoluble material, such as lead, may be used. The current density in this bath is immaterial, since no electrolytic action is desired. The temperature of this bath is between 180 degrees Fahrenheit and 200 degrees Fahrenheit. It has been found that the dark color of the iron or steel is changed in a few seconds to a bright rust-resist-

ing surface, which may be ground or polished with ease. The cleaned part is then dipped into hot water, which removes most of the caustic from the steel surface and leaves the surface dry after a brief exposure in the air.

While some departure from the conditions of temperature, current density and strength of solutions is permissible, it has been found that the best results are obtained in accordance with the above disclosure. In practice, the first bath has acid added thereto at regular intervals to compensate for the loss of acid and maintain the strength of solution. After a while, the amount of iron in the solution becomes so great that it is advisable to throw out the entire solution and start anew. The solution in the third bath is not appreciably affected by use and need only be freshened at intervals to clean the solution from suspended iron particles.

This process has been successfully applied to both iron and steel. As practiced, it results in substantially no etching and leaves a surface clean enough even for immediate soldering. It is important that the cleaned article be taken out of the first bath promptly upon the removal of the scale. While short periods of time in excess of that required for scale removal will not cause any appreciable etching, prolonged stays in the first bath will result in damage.

I claim:

1. A process of removing scale from iron or steel in connection with the preparation of hardened machine parts having scaly surfaces as the result of such hardening and which surfaces are to be prepared for trueing operations while preventing hydrogen embrittlement and pitting within the limits of said trueing operations which comprises making such iron or steel the cathode in ten to fifteen per cent sulphuric acid, maintaining the temperature of said acid at 110 to 120 degrees Fahrenheit, providing an anode of substantially insoluble material, and maintaining a current density of between fifty and sixty amperes per square foot of cathode area for a period not in excess of about 12 minutes.

2. The process of claim 1, in which the cleaned article is brightened by thereafter making it the anode in a solution containing sodium hydroxide and trisodium phosphate at a temperature between 180 and 200 degrees Fahrenheit.

3. The process of claim 1, in which the cleaned article is brightened by thereafter making it the anode in a bath containing between two and eight ounces of sodium hydroxide per gallon of

water at a temperature of 180 to 200 degrees Fahrenheit.

4. The process of claim 1, in which the cleaned article is brightened by thereafter making it the anode in a solution containing between two and eight ounces of sodium hydroxide and between two and four ounces of trisodium phosphate per gallon of water, while maintaining the temperature between 180 and 200 degrees Fahrenheit.

10 5. The process of removing scale from iron or steel in connection with the preparation of hardened machine parts having scaly surfaces as the result of such hardening and which surfaces are to be prepared for trueing operations while preventing hydrogen embrittlement and pitting within the limits of said trueing operations, which comprises making said article the cathode in a bath of ten to fifteen per cent sulphuric acid,

5 maintained at a temperature of between 110 and 120 degrees Fahrenheit, and with a current density of between fifty and sixty amperes per square foot of cathode area, with an anode of substantially insoluble material for a period not in excess of about 12 minutes, withdrawing said article from this bath after the removal of the scale, then making said article the anode in a bath containing about four ounces of sodium hydroxide and between two and four ounces of trisodium phosphate per gallon of water, maintained between 180 and 200 degrees Fahrenheit, keeping said article in this bath until the dark surface is brightened, and then removing said article from said bath and dipping it into hot water to remove 10 a portion of the caustic soda. 15

HARRY SCHAGRIN.